



US011603588B1

(12) **United States Patent**  
Anand et al.

(10) **Patent No.:** US 11,603,588 B1  
(45) **Date of Patent:** Mar. 14, 2023

(54) **OXIDATION AND WEAR RESISTANT COATING**

(71) Applicant: **General Electric Company**, Schenectady, NY (US)

(72) Inventors: **Krishnamurthy Anand**, Bangalore (IN); **Surinder Singh Pabla**, Greer, SC (US); **Lacey Lynn Schwab**, Greenville, SC (US); **Biju Dasan**, Bangalore (IN); **Seung-Woo Choi**, South Glastonbury, CT (US); **Sathisha Chikkabikkodu Hanum**, Bangalore (IN); **Ravikiran Kopparthi**, East Godavari (IN); **David Vincent Bucci**, Simpsonville, SC (US)

(73) Assignee: **General Electric Company**, Schenectady, NY (US)

(\*) Notice: Subject to any disclaimer, the term of this patent is extended or adjusted under 35 U.S.C. 154(b) by 0 days.

(21) Appl. No.: **17/461,136**

(22) Filed: **Aug. 30, 2021**

(51) **Int. Cl.**

**C23C 4/18** (2006.01)  
**F01D 25/24** (2006.01)  
**C23C 4/11** (2016.01)  
**C23C 4/073** (2016.01)  
**F01D 25/00** (2006.01)

(52) **U.S. Cl.**

CPC ..... **C23C 4/18** (2013.01); **C23C 4/073** (2016.01); **C23C 4/11** (2016.01); **F01D 25/00** (2013.01); **F01D 25/24** (2013.01); **F05D 2300/121** (2013.01); **F05D 2300/17** (2013.01); **F05D 2300/2112** (2013.01); **F05D 2300/605** (2013.01)

(58) **Field of Classification Search**

CPC ..... C23C 4/18; C23C 4/073; C23C 4/11; F01D 25/00; F01D 25/24; F05D 2300/121; F05D 2300/17; F05D 2300/2112; F05D 2300/605

See application file for complete search history.

10 ↘



(56)

**References Cited**

**U.S. PATENT DOCUMENTS**

|              |      |         |               |              |
|--------------|------|---------|---------------|--------------|
| 8,202,574    | B2 * | 6/2012  | Carlin .....  | C23C 16/4488 |
|              |      |         |               | 427/252      |
| 2008/0241527 | A1 * | 10/2008 | De Iaco ..... | F04D 29/444  |
|              |      |         |               | 428/339      |
| 2016/0186768 | A1 * | 6/2016  | De Iaco ..... | F04D 29/444  |
|              |      |         |               | 415/173.4    |
| 2017/0024252 | A1 * | 1/2017  | Bacos .....   | C23C 4/134   |
| 2017/0096906 | A1   | 4/2017  | Werner .....  |              |
| 2019/0024251 | A1 * | 1/2019  | Li .....      | C25D 1/02    |
| 2020/0056277 | A1 * | 2/2020  | Kim .....     | C22C 45/08   |

**FOREIGN PATENT DOCUMENTS**

|    |         |    |         |
|----|---------|----|---------|
| EP | 1464723 | A2 | 10/2004 |
| EP | 0919639 | B1 | 2/2005  |

**OTHER PUBLICATIONS**

European Search Report; EP Application No. EP22190131; dated Nov. 22, 2022.

\* cited by examiner

*Primary Examiner* — Igor Kershteyn

(74) *Attorney, Agent, or Firm* — Fletcher Yoder, PC

(57)

**ABSTRACT**

A method includes applying a material coating on a surface of a machine component using a thermal spray, wherein the material coating is formed from a combination of a hard-facing material and aluminum-containing particles. The method also includes thermally treating the material coating to generate an oxide layer comprising aluminum from the aluminum-containing particles, wherein the oxide layer is configured to reduce oxidation of the hardfacing material.

**12 Claims, 4 Drawing Sheets**



FIG. 1



FIG. 2



FIG. 3A



FIG. 3B



FIG. 4A



FIG. 4B

## OXIDATION AND WEAR RESISTANT COATING

### BACKGROUND

The subject matter disclosed herein relates to forming a material coating with oxidation and mechanical wear resistance using a thermal spray process.

A gas turbine, or gas turbine engine, may include an air intake section, a compressor section, a combustion section, a turbine section, and an exhaust section. In operation, the air intake section receives an intake air from the ambient environment, and the compressor section compresses the intake air. The compressed air flows to the combustion section, which uses the compressed air for combustion of one or more fuels to generate a hot combustion gas. The hot combustion gas drives rotation of the turbine section, which in turn drives the compressor section and one or more loads, such as a generator.

During operation of the gas turbine, the components of the gas turbine may be subjected to a variety of conditions (e.g., mechanical contact, relatively high temperatures during combustion, and relatively low temperatures) that may cause wear to the components. For example, bucket interlocks of the gas turbine may be subjected to high temperature (e.g., greater than 500° C., 600° C., 700° C., 800° C., 900° C., and the like) fretting motion, such as when the respective buckets lock up due to centrifugal and aerodynamic forces. Further, the bucket interlocks may be subjected to relatively low temperature (e.g., ambient temperature) fluttering (e.g., during startup of the gas turbine), which may cause mechanical contact along the bucket interlocks. Certain components (e.g., bucket interlocks) may include a coating that reduces the mechanical resistance of the component during certain portions of the operation. The coating may form an oxide layer at the relatively high temperatures disclosed above.

### BRIEF DESCRIPTION

Certain embodiments commensurate in scope with the originally filed claims are summarized below. These embodiments are not intended to limit the scope of the present technology, but rather these embodiments are intended only to provide a brief summary of possible forms of the technology. Indeed, the present system and method may encompass a variety of forms that may be similar to or different from the embodiments set forth below.

In certain embodiments a method includes applying a material coating to a surface of a machine component using a thermal spray, wherein the material coating is formed from a combination of a hardfacing material and aluminum-containing particles. The method also includes thermally treating the material coating to generate an oxide layer comprising aluminum from the aluminum-containing particles, wherein the oxide layer is configured to reduce oxidation of the hardfacing material.

In certain embodiments, a machine component includes a material coating. The material coating includes a layer comprising a first plurality of phases of a hardfacing material and a second plurality of phases of an aluminum-based material. The aluminum-based material is configured to oxidize to reduce beta depletion of the hardfacing material.

In certain embodiments, a machine component comprises a material coating. The material coating includes a first layer comprising a hardfacing material and an aluminum-based material, wherein the first layer is formed by thermal spray

of the hardfacing material and the aluminum-based material. The material coating also includes a second layer formed by heat treatment of the first layer. The second layer has crystalline intermetallic phases of the aluminum-based material.

### BRIEF DESCRIPTION OF THE DRAWINGS

These and other features, aspects, and advantages of the present disclosure will become better understood when the following detailed description is read with reference to the accompanying drawings in which like characters represent like parts throughout the drawings, wherein:

FIG. 1 is a flow diagram of an embodiment of a process for producing an oxidation and mechanical wear resistant (OMWR) coating, in accordance with the present disclosure;

FIG. 2 is a schematic diagram of an embodiment of a deposition system for producing the OMWR coating, in accordance with the present disclosure;

FIG. 3A is a cross-sectional view of an embodiment of a material coating formed without an oxidation wear resistant (OWR) material, in accordance with the present disclosure;

FIG. 3B is a cross-sectional view of an embodiment of an OMWR coating having an oxide layer formed by an oxidation wear resistant material, in accordance with the present disclosure;

FIG. 4A is a schematic diagram of an embodiment of a material coating formed without the OWR material, in accordance with the present disclosure; and

FIG. 4B is a schematic diagram of an embodiment of an OMWR coating having an oxide layer formed by an oxidation wear resistant material, in accordance with the present disclosure.

### DETAILED DESCRIPTION

One or more specific embodiments of the present disclosure will be described below. In an effort to provide a concise description of these embodiments, all features of an actual implementation may not be described in the specification. It should be appreciated that in the development of any such actual implementation, as in any engineering or design project, numerous implementation-specific decisions must be made to achieve the developers' specific goals, such as compliance with system-related and business-related constraints, which may vary from one implementation to another. Moreover, it should be appreciated that such a development effort might be complex and time consuming, but would nevertheless be a routine undertaking of design, fabrication, and manufacture for those of ordinary skill having the benefit of this disclosure.

When introducing elements of various examples of the present disclosure, the articles "a," "an," "the," and "said" are intended to mean that there are one or more of the elements. The terms "comprising," "including," and "having" are intended to be inclusive and mean that there may be additional elements other than the listed elements. Additionally, it should be understood that references to "one example" or "an example" of the present disclosure are not intended to be interpreted as excluding the existence of additional examples that also incorporate the recited features.

In the present context, the term "about" or "approximately" is intended to mean that the values indicated are not exact and that the actual value may vary from those indicated in a manner that does not materially alter the operation concerned. For example, the term "about" or "approxi-

mately" as used herein is intended to convey a suitable value that is within a particular tolerance (e.g.,  $\pm 10\%$ ,  $\pm 5\%$ ,  $\pm 1\%$ ,  $\pm 0.5\%$ ), as would be understood by one skilled in the art.

As generally discussed above, one or more components of a gas turbine may include a material coating that enhances the mechanical wear resistance of the component. When the components of the gas turbine operate at relatively high temperatures (e.g., greater than 500° C., 600° C., 700° C., 800° C., 900° C., and the like), such while the components are exposed to combustion gases, a portion of the material coating may oxidize to form an oxide layer.

The present disclosure is directed to techniques for improving the longevity of a machine component (e.g., a component of a gas turbine) by combining an oxidation wear resistant (OWR) material with a mechanical wear resistant (MWR) material and depositing the combination or mixture of the materials onto a surface of the component via a thermal spray technique to produce an oxidation and mechanical wear resistant (OMWR) coating. As discussed in more detail herein, the OWR material may block, reduce, or mitigate oxidation of the MWR material. For example, the OWR material may include aluminum-based material(s) (e.g., aluminum, aluminum oxide, CoNiCrAlY particles, or both) that form an OWR oxide layer, which is a self-limiting oxide layer. That is, when oxygen is present, at least a portion of the aluminum (e.g., originating from the aluminum-based material(s) of the OWR material) in the OMWR coating may oxidize to form the OWR oxide layer that terminates after a few microns (i.e., micrometers) (e.g., approximately 10 microns, less than 10 microns, approximately 5 microns). A thickness of the self-limiting oxide layer may be less than a thickness of an oxide layer formed by a material that does not readily produce a self-limiting oxide layer, such as the MWR material. Moreover, the OWR oxide layer may also reduce a rate of consumption of the MWR material by reducing oxidation and subsequent erosion of the MWR material, while maintaining a relatively small thickness of the coating. Accordingly, utilizing the OMWR coating may reduce operational costs associated with reapplication of a worn coating and/or replacement of a worn component. It is noted that by the OMWR coating forming the OWR oxide layer, which is self-limiting, the OMWR coating may have improved longevity as compared to certain existing coatings. For example, because the OWR oxide layer is self-limiting, less of the OWR oxide layer forms, and thus, less of the OWR material is consumed. Further, the OWR oxide layer may prevent beta depletion of the MWR material within in the OMWR coating. Accordingly, a component coated with the OMWR material that is repeatedly subjected to the relatively high temperatures may erode more slowly than components coated with certain existing coatings. As the OMWR material erodes more slowly, the component coated with the OMWR material is provided with mechanical wear resistance for a longer duration.

With this in mind, FIG. 1 is a flow diagram of an embodiment of a process 10 for producing an OMWR coating 12 on a substrate 14 (e.g., a machine component) that enhances mechanical wear resistance and oxidation resistance of the substrate 14. As described herein, the substrate 14 may be a component of a gas turbine, such as part of a combustion section, bucket, bucket interlock, or another component of the gas turbine that may be subjected to relatively high temperatures (e.g., greater than 800° C.) and mechanical contact during operation. The steps illustrated in the process 10 are meant to facilitate discussion and are not intended to limit the scope of this disclosure, because

additional steps may be performed, certain steps may be omitted, and the illustrated steps may be performed in an alternative order or in parallel, where appropriate.

To start the process 10, at block 16, an OWR material 18 and an MWR material 20 are deposited onto, applied to, formed integrally with (e.g., during manufacture), or otherwise coupled to the substrate 14, such as to one or more surfaces of the substrate 14. The OWR material 18 is generally a material that forms a self-limiting oxide layer that is a solid at relatively high temperatures (e.g., greater than 800° C. The OWR material may include certain aluminum-based material(s). Certain non-limiting examples of such aluminum-based material(s) include aluminum, aluminum oxide, and aluminum alloy(s) (e.g., CoNiCrAlY). The OWR material 18 may include micron-sized particles, nanoparticles, or larger-sized particles, of the aluminum based material(s). In some embodiments, the OWR material 18 consists essentially of aluminum (e.g., as a metal, intermetallic, or alloy) or alumina (e.g., aluminum oxide).

The MWR material 20 may include a hardfacing material, whether a micron-sized particle, nanoparticle, or larger size particle. In general, hardfacing materials including metals that deposited (e.g., using thermal spray) to impact improved hardness to a surface underneath. The hardfacing material may include transition metal carbide(s), e.g., including carbide(s) with chromium, tungsten, vanadium, molybdenum, other suitable element(s), or a combination thereof. Additionally or alternatively, the hardfacing material may include certain transition metal alloy(s), including cobalt alloy(s), molybdenum alloy(s), chromium alloy(s), nickel alloy(s), other suitable alloy(s), or a combination thereof. For example, the MWR material may have a general composition of M-Mo—Cr—Si (M=Co or Ni), such as Tribaloy® (e.g., T800 or Co800 particles) from Deloro Stellite Holdings Corporation, a Kennametal Company. In an embodiment where the OWR material 18 and/or the MWR material 20 are particles (e.g., micron-sized particles, nanoparticles, or larger particles), the particles may have a distribution of shapes. For example, the OWR material 18 may include micron-sized particles that are 10%, 20%, 30%, 40%, 50%, 60%, 70%, 80% 90%, or 95% spherical, and the MWR material 20 may include nano-size particles that are 10%, 20%, 30%, 40%, 50%, 60%, 70%, 80% 90%, or 95% spherical. At least in some instances, the combination of particle shape (e.g., spherical) and different size distributions may improve the properties of the result OMWR coating 12 discussed herein.

The OMWR coating 12 may include different phases formed from the OWR material 18 and the MWR material 20, as discussed in more detail with respect to FIGS. 4A and 4B. For example, in an embodiment in which the MWR material 20 includes Co—Mo—Cr—Si, the OMWR coating 12 formed by the deposition of the OWR and MWR materials may include a Co—Mo—Si phase, a Co-matrix, and Cr-containing regions. In embodiments in which the OWR material 18 includes aluminum oxide, the OMWR coating may include phase(s) of alumina, such as gamma phase and/or beta phase.

In some embodiments, the OWR material 18 and the MWR material 20 may be deposited onto the one or more surfaces of the substrate 14 using a thermal spray process, such as high velocity oxygen fuel (HVOF) thermal spray, high velocity air fuel (HVAF) spray, and the like, which is discussed in more detail with respect to FIG. 2. In some embodiments, the OWR material 18 and the MWR material 20 may be deposited onto the one or more surfaces of the substrate 14 using deposition methods such as air plasma

spray, cored-wire arc wire spray, and the like. In some embodiments, the OWR material **18** and the MWR material **20** may be deposited as a mixture of the OWR material **18** and the MWR material **20**. That is, the OWR material **18** may be blended with the MWR material **20**. For example, the mixture may include 30% by weight of the OWR material **18** and 70% by weight of the MWR material **20**, 50% by weight of the OWR material **18** and 50% by weight of the MWR material **20**, or 70% by weight of the OWR material **18** and 30% by weight of the MWR material **20**. At least in some instances, using less of the OWR material **18** may provide more wear resistance (e.g., both oxidation resistance and wear resistance). For example, an OMWR coating **12** formed using 30% by weight of the OWR material **18** and 70% by weight of the MWR material **20** may provide increased oxidation resistance than an OMWR coating **12** formed using 70% by weight of the OWR material **18** and 30% by weight of the MWR material **20**.

In some embodiments, the OWR material **18** and the MWR material **20** may be deposited onto the substrate **14** (e.g., using a thermal spray) separately. For example, the MWR material **20** may be deposited and, subsequently, the OWR material **18** may be deposited on top of the MWR material **20**. As such, the resulting OMWR coating **12** may have a first layer including the MWR material **20** in contact with the substrate, and a second layer including the OWR material **18**. At least in some instances, an intermediate layer (e.g., between the first layer and the second layer) may form that includes both the OWR material **18** and the MWR material **20**. It should be noted that, at least in some instances, the OWR material **18** and the MWR material **20** may be deposited multiple times on the substrate **14**, such as depositing alternating layers of the OWR material **18** and the MWR material **20** and/or depositing multiple layers using the same material (e.g., the OWR material **18** or the MWR material **20**).

The mixture or combination of the OWR material **18** and the MWR material **20** deposited onto the substrate **14** (e.g., using a thermal spray) produces the OMWR coating **12**. At block **22**, the OMWR coating **12** is thermally treated (e.g., heated) to generate an OWR oxide layer **24**. The OWR oxide layer **24** may include an aluminum-based oxide layer that provides oxidation wear resistance to a mechanical wear resistant layer that includes a combination of the OWR material and the MWR material. Thermally treating the OMWR coating **12** includes heating the OMWR coating **12** (e.g., the substrate **14** or component that includes the OMWR coating **12**) to a relatively high temperature, such as approximately 500° C., approximately 600° C., approximately 700° C., approximately 800° C., greater than 800° C. for a predetermined time period. The predetermined time period may be 1 hour, 5 hours, 10 hours, 20 hours, or greater than 20 hours. At least in some instances, thermally treating the OMWR coating **12** may include heating the OMWR coating **12** in a furnace capable of reaching the relatively high temperature. In some embodiments, thermally treating the OMWR coating **12** may include operating the machine (e.g., the gas turbine) with one or more surfaces of the component of the machine coated with the OMWR coating, and thus facilitating formation of the OWR oxide layer **24** during operation.

In some embodiments, the OMWR coating **12** (e.g., and the substrate **14** coated with the OMWR coating) may be pre-heat treated, which may precipitate sub-micrometric crystalline intermetallic phases (e.g., from the OWR material and/or the MWR material) present in the OMWR coating **12**. That is, before thermally treating the OMWR

coating **12** to grow the OWR oxide layer **24** on the OMWR coating **12**, the OMWR coating **12** may be heated at a relatively lower temperature and/or in the presence of an inert gas or relatively oxygen-free environment. For example, in embodiments in which the OMWR coating **12** includes an aluminum-based material (e.g., the OMWR coating **12** includes an alumina phase originally from the deposited OWR material **18**), pre-heat treatment may produce a continuous aluminum scale at the surface of the OMWR coating **12**, which may be below the solution and age heat treatment of the alloy. The aluminum scale formed by pre-heat treatment may establish improved wear properties at temperatures greater than approximately 900° C.

In certain embodiments, the MWR material **20** may include Co800 particles, and the OWR material may include an aluminum-based alloy, such as CoNiCrAlY particles. In such embodiments, at block **16**, the Co800 particles and the CoNiCrAlY particles may be deposited using the HVOF process. The resulting OMWR coating **12** may include Co800 regions (e.g., splats) that are proximate to at least one source of aluminum from the CoNiCrAlY particles (e.g., within the diffusion distance of the aluminum at a temperature greater than 1500 F). When the OMWR coating **12** is exposed to a relatively high temperature, a relatively thin layer of aluminum oxide based thermally grown oxide (TGO) (i.e., the OWR oxide) is formed (e.g., less than 5 microns thick after 2000 hours of exposure at 1700 F to 1800 F) that provides oxidation protection. Because the resulting oxide scale (e.g., the OWR oxide layer **24**) is relatively thin (e.g., less than 10 microns), the oxide scale may be flexible so that the oxide layer does not crack (i.e., in response to contact with the oxide scale and another surface or due to a difference between thermal expansion coefficients of the oxide scale and the material layer below) cushioned by tougher metal underneath during impact and continue to provide protection to the layer(s) below, including the MWR material **20**. Because the presence of the OWR material causes a thinner oxide layer (i.e., the OWR oxide layer) to form, even if the oxide scale is removed after subsequent oxidation and wear, the OMWR coating **12** may have greater longevity than a material coating formed without the OWR material **18**, thereby increasing the service life of the component. The material combination disclosed herein develops a thin and protective aluminum oxide scale, which reduces degradation mechanisms, such as beta depletion of the CoNiCrAlY phase.

In another embodiment, the OWR material **18** may include a mixture of particles. For example, the OWR material **18** may include a mixture of CoNiCrAlY particles and aluminum oxide particles. Using both CoNiCrAlY and aluminum oxide may improve the wear resistance of the material. For example, the OWR oxide layer formed by the aluminum oxide may reinforce the wear resistance of the OWR oxide layer formed by the aluminum present in the CoNiCrAlY. This material combination develops a thin and protective aluminum oxide scale (i.e., the OWR oxide layer), which reduces degradation mechanisms, such as beta depletion of the CoNiCrAlY phase. The mixture may be thermal sprayed onto the substrate **14**. At least in some instances, the thermal spraying includes an HVOF process in which the aluminum oxide is soft or semi-molten within the HVOF plume, thereby resulting in the aluminum oxide becoming entrapped within the CoNiCrAlY phase. At least in some instances, the high temperature plume may reinforce the CoNiCrAlY particle deposited on the substrate, thereby forming a wear resistant composite.

In some embodiments, at least one of the OWR material **18** or the MWR material **20** may include particles having different size distributions. For example, the OWR material **18** may include a first plurality of aluminum oxide particles having a nano-size distribution (e.g., having an average diameter of approximately 5 nm, 10 nm, 50 nm, 100 nm, 200 nm, 500 nm, and the like). Additionally, the OWR material **18** may include a second plurality of aluminum oxide particles having a micro-size distribution (e.g., having an average diameter of approximately 1  $\mu$ m, 5  $\mu$ m, 10  $\mu$ m, 50  $\mu$ m, 100  $\mu$ m, 200  $\mu$ m, 500  $\mu$ m, and the like).

In some embodiments, both the OWR material **18** and the MWR material **20** may include particles having different size distributions. That is, the OWR material **18** may include particles of a first size distribution and the MWR material **20** may include particles having a second size distribution. For example, the OWR material **18** may include CoNiCrAlY particles and the MWR material may include aluminum oxide. The OWR materials **18** may have a micron-size distribution and the MWR material **20** may have a nano-size distribution. In some embodiments, the OWR materials **18** may have a nano-size distribution and the MWR material **20** may have a micron-size distribution. At least in some instances, a bimodal size distribution may improve wear resistance. In an embodiment where the OWR material **18** and the MWR material **20** include particles having different size distributions, the mixture of the particles may vary. For example, the mixture may include 10%, 20%, 30%, 40%, 50%, 60%, 70%, and the like, by weight, of the OWR material **18** and 90%, 80%, 70%, 60%, 50%, 40%, 30%, and the like, by weight, of the MWR material **20**.

As discussed above, the oxidation wear resistant material and the mechanical wear resistant material may be deposited onto the component using a thermal spray technique, such as HVOF. To illustrate this, FIG. 2 is a schematic diagram of an embodiment of a deposition system for producing the OMWR coating. In the illustrated embodiment, the deposition system includes an HVOF thermal spray system **26** for applying the OMWR coating **12** onto the substrate **14** (e.g., bucket interlock, in certain embodiments). At least in some instances, HVOF thermal deposition of certain materials, such as hardfacing materials, may result in the formation of certain Laves phases that provide increased mechanical wear resistance to a coating (e.g., the OMWR coating **12**). Examples of such Laves phases are described herein with respect to the alloy regions of FIGS. 4A and 4B.

As illustrated, in certain embodiments, the HVOF thermal spray system **26** includes a thermal spray device **28** having a nozzle **30** at an axial end of the thermal spray device **28**, a fuel gas channel **32** extending axially through the thermal spray device **28**, one or more air channels **34** extending axially through the thermal spray device **28** and the nozzle **30**, and a material coating precursor inlet **36** extending radially inward through the thermal spray device **28** to the fuel gas channel **32**. The thermal spray device **28** is described herein as being an HVOF thermal spray device insofar as air is mixed with fuel. However, in other embodiments, the thermal spray device **28** may be an HVOF thermal spray device insofar as oxygen, instead of air, may be mixed with fuel.

In operation, air (or oxygen, in certain embodiments) is provided to the air channel(s) **34** (e.g., via an air inlet) and fuel (e.g., liquid and/or gas fuel, such as kerosene, hydrogen, methane, propane, propylene, acetylene, natural gas, and the like) is provided to the fuel gas channel **32** (e.g., via a fuel inlet). The air and fuel are mixed and subsequently ignited (e.g., via an ignition source, such as an ignition plug, within

the nozzle **30**, in certain embodiments) and combusted to produce a high pressure (e.g., less than or approximately equal to 1 MPa) and hot (e.g., approximately 1500° C.) gas. Additionally, the material coating precursor (e.g., the OWR material **18**, the MWR material **20**, or both) is provided to the material coating precursor inlet **36** (e.g., as a solid particle powder, in certain embodiments) to be added to the fuel gas stream upstream of the nozzle **30**, which produces a high pressure and hot gas from the resulting combusting air, fuel, and powder mixture. The material coating precursor, when in contact with the high pressure and hot gas, is accelerated to a high velocity (e.g., between approximately 1000 m/s to 1500 m/s, in certain embodiments) and may be at least partially melted, thereby producing a material spray **38** that exits out of the nozzle **30**, and deposits onto a surface of the substrate **14**.

As discussed herein, the OMWR coating **12** may form an OWR oxide layer **24** that reduces erosion of the OMWR coating **12**. To illustrate the OMWR coating **12**, FIGS. 3A 20 and 3B are cross-sectional views of an embodiment of a deposited MWR material coating **40** that does not include OWR material **18** and an embodiment of a deposited OMWR material coating **12** that includes the OWR oxide layer **24**, respectively, and each coating includes an oxide layer formed from the material(s) disposed onto the substrate.

In FIG. 3A, the deposited MWR material coating **40** has an MWR oxide layer **44**, which may be formed after exposure to a relatively high temperature (e.g., greater than 30 1500 F). As described herein, the MWR oxide layer **44** may be less wear resistant than the material present in the MWR deposition layer **46**. Accordingly, the MWR oxide layer **44** may erode after forming due to mechanical contact with another object. It should be noted that an additional MWR oxide layer may form after subsequent exposure of the MWR deposition layer **46** to relatively high temperatures. Accordingly, repeated formation of the MWR oxide layer **44** may gradually erode the MWR material coating **40** due to beta depletion mechanisms. As shown in FIG. 3A, the MWR oxide layer **44** has a thickness **48** of approximately 20 microns, which may be relatively thicker than an oxide layer formed using an OWR material, as discussed herein. It should be noted that the substrate (not shown) is generally below the MWR coating **40** and the MWR oxide layer **44** forms above the MWR coating **40**.

FIG. 3B is a cross-sectional view of an embodiment of an OMWR coating **12** deposited on a substrate (e.g., the substrate **14**) having an OWR oxide layer **24** formed by the OWR material on top of the OMWR coating **12**. As 50 described herein, the OWR oxide layer **24** may be self-limiting, and thus while the OWR oxide layer **24** may erode after forming (e.g., due to mechanical wear at relatively low and/or relatively high temperatures), less of the OWR material may be consumed during subsequent exposure of the 55 OMWR coating **12** to relatively high temperatures (e.g., as compared to the embodiment of FIG. 3A). Accordingly, the OMWR coating **12** may provide mechanical wear resistance to the substrate (e.g., the bucket interlocks) for a relatively longer period of time than the MWR material coating 60 disclosed above with reference to FIG. 3A. As also shown in FIG. 3B, the thickness **50** of the OWR oxide layer **24** is less than 10 microns, and thus thinner than the oxide layer formed on the MWR material of the coating of FIG. 3A. As 65 discussed herein, the OWR oxide may be a material that forms a self-limiting oxide layer that may not continue to grow in certain conditions (e.g., temperature and pressure) beyond a certain thickness. Accordingly, less of the material

used to form the OMWR coating 12 is consumed each time the OWR oxide layer 24 is formed. FIG. 3B also includes an inset cross-sectional view 52 of the OMWR coating 12. As shown, an additional oxide layer 54 is present on the OWR oxide layer 24. The additional oxide layer 54 may be formed of the MWR material present in the OMWR coating 12. For example, in an embodiment in which the MWR material 20 is a cobalt or chromium-based alloy and is used to produce the OMWR coating 12, the additional oxide layer 54 may include cobalt oxide and/or chromium oxide. The additional layer 54 is relatively thin compared to the oxide layer of FIG. 3A that is formed without the OWR material, and thus, less of the MWR material used to produce the OMWR coating 12 is consumed by the oxidation process.

As discussed herein, the OMWR coating 12 may include regions formed from the OWR material 18 and the MWR material 20. To illustrate this, FIGS. 4A and 4B are schematic diagrams of an embodiment of an MWR material coating 56 (e.g., material coating formed without OWR material) and an embodiment of an OMWR material coating 12 (e.g., having an OWR oxide layer formed by the OWR material), respectively. In the illustrated embodiment, the MWR material 20 of the MWR coating 56 and the OMWR material coating 12 includes Co—Mo—Si—Cr. As shown in FIG. 4A, the MWR material coating 56 includes a material oxide scale region 60 having a first thickness 62, which may include cobalt, chromium, and oxides of both. The MWR material coating 56 also includes a matrix region 64 which may be a cobalt-matrix, an alloy region 66, which may include a Co—Mo—Si phase, and an oxidized alloy region 68, which may include oxidized Co—Mo—Si.

Turning to FIG. 4B, the OMWR material coating 12 includes a material oxide scale region 60 having a thickness 70 that is smaller than the thickness of the material oxide scale region of the MWR material coating of FIG. 4A, which may indicate that less MWR material is consumed as a result of the oxide (i.e., the OWR oxide layer) forming. Below the self-limiting oxide layer 72, the OMWR material coating 12 includes a beta depletion zone 74, a gamma matrix region 76, a beta phase region 78, an alloy region 66, and an oxidized alloy region 80. The gamma matrix region 76 and the beta phase region 78 may be formed of the OWR material, and thus may include aluminum oxide. Accordingly, at least a portion of these regions may be eroded upon oxidation and formation of the self-limiting oxide layer 72.

While the OMWR material coating 12 includes the oxidized alloy region 80, there is less of the oxidized alloy region 80 as compared to an amount of the oxidized alloy region 68, shown in FIG. 4A. Thus, this indicates there is less erosion of the regions resulting from the MWR material 20 in the OMWR material coating as compared to the MWR material coating 56.

FIG. 4B illustrates different regions that may form within the OMWR coating 12 discussed herein. As discussed herein, the coating (e.g., the OMWR material coating 12 and the MWR coating 56) may include various Laves phases. For example, in embodiments in which the MWR material includes a Co—Mo—Cr—Si material, the alloy region 66 may include such Laves phases as  $\text{Co}_2\text{Mo}_3\text{Si}$  and  $\text{CoMoSi}$ . As shown in the illustrated embodiment of FIG. 4B, the alloy regions 66 are dispersed among the gamma matrix region 76.

Accordingly, the present disclosure relates to an OMWR coating that enhances oxidation wear resistance and mechanical wear resistance of a component, such as a component of a gas turbine, that may be subjected to relatively high temperatures (e.g., greater than 1500 F) and

relatively low temperatures (e.g., ambient temperature, less than 1500 F) during operation. The OMWR coating may reduce or eliminate the formation of relatively thick oxides (e.g., oxide scales), and thus reduce a rate of erosion of the OMWR coating, thereby enabling the component to be utilized for longer periods of time. In some embodiments, the OMWR coating is formed by thermal spraying a mixture of a first material and a second material onto a substrate. The first material (e.g., the MWR material 20) may have a relatively high mechanical wear resistance, and the second material (e.g., the OWR material 18) may have a relatively high oxidation resistance. At least in some instances, the second material may form a self-limiting oxide layer. As discussed herein, the self-limiting oxide may reduce the rate at which the material forming the OMWR coating is consumed. In this way, the OWR material may reduce the consumption of the MWR material due to oxidation, thereby increasing the longevity of the component coated with the OMWR coating. Moreover, although the OMWR coating includes two materials (e.g., the MWR material and the OWR material), the thickness of the OMWR coating may be relatively thin (e.g., less than 10 microns), and thus may not significantly alter the dimensions of the component.

Accordingly, technical effects of this disclosure include, and are not limited to, improving the oxidation wear resistance of a coating applied to a substrate. By improving the oxidation wear resistance of the coating, the coating is less likely to oxidize, and therefore form a material that may have a relatively lower mechanical wear resistance thereby improving the longevity of the coating. The machine components, such as bucket interlocks of a gas turbine, that are coated with an OMWR coating may have increased wear resistance while operating at a broad range of temperatures.

This written description uses examples to disclose the subject matter, including the best mode, and also to enable any person skilled in the art to practice the subject matter, including making and using any devices or systems and performing any incorporated methods. The patentable scope of the subject matter is defined by the claims and may include other examples that occur to those skilled in the art. Such other examples are intended to be within the scope of the claims if they have structural elements that do not differ from the literal language of the claims, or if they include equivalent structural elements with insubstantial differences from the literal language of the claims.

The techniques presented and claimed herein are referenced and applied to material objects and concrete examples of a practical nature that demonstrably improve the present technical field and, as such, are not abstract, intangible or purely theoretical. Further, if any claims appended to the end of this specification contain one or more elements designated as "means for [perform]ing [a function] . . ." or "step for [perform]ing [a function] . . .", it is intended that such elements are to be interpreted under 35 U.S.C. 112(f). However, for any claims containing elements designated in any other manner, it is intended that such elements are not to be interpreted under 35 U.S.C. 112(f).

Further aspects of the invention are provided by the subject matter of the following clauses:

1. A method, comprising: applying a material coating to a surface of a machine component using a thermal spray, wherein the material coating is formed from a combination of a hardfacing material and aluminum-containing particles; and thermally treating the material coating to generate an oxide layer comprising aluminum from the aluminum-containing particles, wherein the oxide layer is configured to reduce oxidation of the hardfacing material.

## 11

2. The method of any preceding clause, wherein the hardfacing material comprises particles having a first size distribution and wherein the aluminum-containing particles have a second size distribution, wherein the first size distribution is different than the second size distribution.

3. The method of any preceding clause, wherein the oxide layer has a thickness of less than 10 microns.

4. The method of any preceding clause, wherein the aluminum-containing particles consist essentially of aluminum.

5. The method of any preceding clause, wherein the hardfacing material comprises M—Mo—Cr—Si, where M comprises Ni or Co.

6. The method of any preceding clause, wherein the oxide layer comprises crystalline intermetallic phases formed by a pre-heat treatment of the material coating.

7. The method of any preceding clause, wherein thermally treating the material coating comprises heating the material coating to approximately 800° C.

8. The method of any preceding clause, wherein applying the material coating comprises depositing semi-molten aluminum oxide to the surface while the material coating is applied to the surface.

9. A machine component comprising a material coating, wherein the material coating comprises: a layer comprising a first plurality of phases of a hardfacing material and a second plurality of phases of an aluminum-based material, wherein the aluminum-based material is configured to oxidize to reduce beta depletion of the hardfacing material.

10. The machine component of any preceding clause, wherein the machine component comprises a gas turbine component.

11. The machine component of any preceding clause, wherein the hardfacing material comprises a transition metal alloy.

12. The machine component of any preceding clause, wherein the aluminum-based material comprises aluminum before oxidation.

13. The machine component of any preceding clause, wherein the aluminum-based material is configured to form an aluminum oxide layer, wherein the material coating comprises the aluminum oxide layer.

14. The machine component of any preceding clause, wherein the aluminum oxide layer has a thickness of less than 20 microns.

15. The machine component of any preceding clause, wherein the aluminum-based material comprises CoNiCrAlY particles, aluminum oxide before oxidation, or both.

16. The machine component of any preceding clause, wherein the aluminum-based material comprises a mixture of aluminum oxide before oxidation and CoNiCrAlY particles.

17. A machine component comprises a material coating, the material coating comprising a first layer comprising a hardfacing material and an aluminum-based material, wherein the first layer is formed by thermal spray of the hardfacing material and the aluminum-based material; and a

## 12

second layer formed by heat treatment of the first layer, wherein the second layer comprises crystalline intermetallic phases of the aluminum-based material.

18. The material coating of any preceding clause, wherein the thermal spray comprises high velocity oxygen-fuel (HVOF) thermal spray.

19. The material coating of any preceding clause, wherein the hardfacing material comprises M—Mo—Cr—Si, where M comprises Ni or Co.

20. The material coating of any preceding clause, wherein the hardfacing material comprises CoNiCrAlY particles.

The invention claimed is:

1. A machine component comprising a material coating, wherein the material coating comprises:

15 a layer comprising a first plurality of phases of a hardfacing material and a second plurality of phases of an aluminum-based material, wherein the aluminum-based material is configured to oxidize to reduce beta depletion of the hardfacing material.

20 2. The machine component of claim 1, wherein the machine component comprises a gas turbine component.

3. The machine component of claim 1, wherein the hardfacing material comprises a transition metal alloy.

4. The machine component of claim 1, wherein the aluminum-based material comprises aluminum before oxidation.

5. The machine component of claim 1, wherein the aluminum-based material is configured to form an aluminum oxide layer, wherein the material coating comprises the aluminum oxide layer.

30 6. The machine component of claim 5, wherein the aluminum oxide layer has a thickness of less than 20 microns.

7. The machine component of claim 1, wherein the aluminum-based material comprises CoNiCrAlY particles, aluminum oxide before oxidation, or both.

8. The machine component of claim 1, wherein the aluminum-based material comprises a mixture of aluminum oxide before oxidation and CoNiCrAlY particles.

40 9. A machine component comprises a material coating, the material coating comprising:

a first layer comprising a hardfacing material and an aluminum-based material, wherein the first layer is formed by thermal spray of the hardfacing material and the aluminum-based material; and

45 a second layer formed by heat treatment of the first layer, wherein the second layer comprises crystalline intermetallic phases of the aluminum-based material.

10. The material coating of claim 9, wherein the thermal spray comprises high velocity oxygen-fuel (HVOF) thermal spray.

11. The material coating of claim 9, wherein the hardfacing material comprises M—Mo—Cr—Si, where M comprises Ni or Co.

50 12. The material coating of claim 9, wherein the hardfacing material comprises CoNiCrAlY particles.

\* \* \* \* \*